

1

3,194,763

## POLYMERIC COMPOSITION AND LUBRICANT CONTAINING IT

Chester D. Gordon, Richmond, Frank A. Stuart, Orinda, and Alfred Goldschmidt, El Cerrito, Calif., assignors to California Research Corporation, San Francisco, Calif., a corporation of Delaware  
No Drawing. Continuation of applications Ser. No. 38,705 and Ser. No. 38,749, June 27, 1960. This application Dec. 18, 1962, Ser. No. 245,409  
2 Claims. (Cl. 252—51.5)

This application is a continuation of Gordon, Stuart and Goldschmidt patent application No. 38,705, filed June 27, 1960; and Goldschmidt, Gordon and Stuart patent application No. 38,749, filed June 27, 1960, both of which applications are now abandoned.

This invention is directed to a novel polymeric composition. More particularly, the invention is concerned with a superior new polymeric composition useful as an ashless detergent for internal combustion engine lubricating oils and as a dispersant for engine fuels and hydrocarbon compositions in general. The polymeric composition of the present invention is also useful as a promoter in grease manufacture for improving the yields of soap thickened greases.

Lubricant compositions are primarily useful in the reduction of friction between rubbing surfaces as in the case of pistons, bearings and other moving parts of engines. In addition, the lubricant compositions prevent the deposit of solid materials on engine surfaces coming in contact with the lubricant composition. Such deposits tend to interfere with normal circulation of the lubricant composition and act as abrasives causing excessive wear of engine parts.

A substantial proportion of modern engine deposits is attributable to the additives commonly present in lubricant compositions, particularly in the case of metal-containing additives. As a lubricant composition is consumed by combustion on cylinder walls and the like in the engine, such metal-containing additives may form an ash which deposits out on the engine surfaces coming into contact with the lubricant composition.

In accordance with the present invention a superior new ashless detergent lubricant composition has been discovered comprising a major portion of an oil of lubricating viscosity and a minor portion sufficient to enhance the detergent characteristics of the composition of an oil-soluble copolymer which comprises (A) at least one oil-solubilizing monomer having a single polymerizable ethylenic group and containing a mono- or divalent hydrocarbon group of from 4 to 30 aliphatic carbon atoms, more particularly, an alkyl ester of an unsaturated monocarboxylic acid of 3 to 5 carbon atoms and (B) at least one oxirane substituted monomer having a single polymerizable ethylenic group and an epoxy group, more particularly, a glycidyl ester of an unsaturated monocarboxylic acid of 3 to 5 carbon atoms the epoxy ring being reacted with an aliphatic polyamine containing at least one nontertiary amino group, the molar ratio of the oxirane portion to amino compound being approximately 1:1, said copolymer containing from about 0.05 to 8.0% by weight of nitrogen and having a total molecular weight of at least about 2,000.

The lubricant composition of this invention as described above is unusually effective in the prevention of engine deposits. The detergent copolymer of the composition contains no metal component and is therefore substantially free of any ash-forming tendencies. This is a particular advantage over conventional detergent

2

lubricant compositions containing organic metal salts to prevent deposits.

The ashless detergent lubricant composition of the present invention is also outstandingly effective in providing detergency over a wide temperature range. It gives excellent performance in relatively low temperature operation such as that encountered in gasoline internal combustion engines operating under "stop and go" city driving conditions. It also functions remarkably well in engine operation involving higher temperatures such as those encountered in diesel engines.

The essential component of the polymeric detergent of the lubricant composition as described above is the predominantly aliphatic hydrocarbon macromolecule having epoxy groups reacted with a single nontertiary amino group of an amino compound to yield an amino-alcohol group. The aliphatic hydrocarbon portion provides the oil-solubility to the copolymer, and the glycidyl-amino compound portion supplies the surface active detergent polarity to the polymer. These oil-solubilizing and polar portions combine in the macromolecule to give the detergent properties as noted above.

In the present description the term "macromolecule" is employed in its commonly accepted sense and refers to large molecules such as those synthesized by polymerization and condensation reactions as well as those occurring in nature, for example, the polysaccharides and the polypeptides illustrated by cellulose and proteins. Most suitably, the predominantly aliphatic hydrocarbon macromolecule detergent additive of the invention is a polymeric type compound. Such compounds may be prepared by first introducing epoxy groups or attaching oxirane groups to ethylene, propylene or isobutylene polymers by means of reactive centers which provide linking groups. Following this, the epoxy groups are reacted with the amino compounds. More satisfactorily for present purposes, however, such polymeric compounds are obtained by copolymerizing the appropriate oil-solubilizing and epoxy substituted monomers as hereinafter described, followed by reaction with the amino compound to give the oil-soluble polymer having the essential polar acting amino-alcohol groups.

The oil-solubilizing monomer portion of the polymeric additives of this invention can be any compound having a single polymerizable ethylenic group together with an oil-solubilizing hydrocarbon group of from 4 to 30 aliphatic carbon atoms. Such monomers are essentially characterized by their ability to copolymerize through said ethylenic group with monomers containing the intermediate epoxy groups or the polar-acting amino-alcohol group referred to above. Alternatively, the oil-solubilizing aliphatic radical can be introduced into the copolymer of the composition according to this invention following the polymerization. This aliphatic radical, whether present in the original monomer or introduced into the copolymer imparts oil-solubility to the polymer. It is preferably a branched or straight chain alkyl radical or a cycloalkyl radical such as butyl, isobutyl, n-pentyl, decyl, dodecyl, cyclohexyl, etc., or an alkenyl radical such as oleyl, ricinoleyl or the like wherein the ethylenic double bond has substantially no copolymerizing tendency.

Oil-solubilizing monomers of this general character are well known in the art and are frequently employed as the oil-solubilizing portion of copolymers which are added to lubricating oils to improve the viscosity index and pour point characteristics thereof. They include such materials as olefins and ethylenically unsaturated ethers and esters and the like.

Representative oil-solubilizing olefins and monomeric compounds of the aforementioned types which can be em-

ployed to form the copolymeric additives of the present invention include the following:

## OLEFINS

|                        |                        |
|------------------------|------------------------|
| Ethylene               | Dodecene-1             |
| Propylene              | Hexadecene-1           |
| Butene-1               | Cyclohexene            |
| Isobutene              | Octadecene-1           |
| Pentene-1              | 4-octylcyclohexene-1   |
| Hexene-1               | 3-phenylhexadecene-1   |
| 2-ethylhexene-1        | p-Octylstyrene         |
| Di- and triisobutylene | Vinyl cyclohexane      |
| Tripropylene           | p-Tertiarybutylstyrene |

## ETHERS

|                                       |                                     |
|---------------------------------------|-------------------------------------|
| Vinyl n-butyl ether                   | Propenyl 2-ethylhexyl ether         |
| Vinyl 2-ethylhexyl ether              | Crotyl n-octyl ether                |
| Allyl n-butyl ether                   | Isopropenyl dodecyl ether           |
| Allyl isobutyl ether                  | 1-decenyl butyl ether               |
| Allyl cyclohexyl ether                | 1-eicosenyl decyl ether             |
| Allyl 4,8,8-tetramethyl dodecyl ether | Vinyl p-octylphenyl ether           |
| Methallyl n-hexyl ether               | Methallyl p-tert. butylphenyl ether |
| Methallyl n-decyl ether               | 1 - decenyl p - cetylphenyl ether   |
| Methallyl 2-ethylhexyl ether          | 1 - decenyl 2 - phenylbutyl ether   |
| Methallyl octadecyl ether             |                                     |

## ESTERS

|                                   |                                           |
|-----------------------------------|-------------------------------------------|
| Vinyl caproate                    | Decyl vinyl acetate                       |
| Vinyl palmitate                   | Isooctyl $\alpha$ -chloroacrylate         |
| Vinyl oleate                      | p-Isoamylphenyl 2-hexadecenoate           |
| Allyl caprylate                   | 4-p-polylbutyl 2-octadecenoate            |
| Allyl laurate                     | Undecyl cinnamate                         |
| Allyl oleate                      | Methylcyclohexyl 2-ethyl-2-hexenoate      |
| Allyl palmitate                   | 5-ethyldecosyl crotonate                  |
| Allyl stearate                    | Octadecyl isocrotonate                    |
| Allyl 2-ethylhexanoate            | n-Butyl 2-eicosenoate                     |
| Allyl ricinoleate                 | p-Tert. amylophenyl octadecyl maleate     |
| Allyl esters of babassu acids     | p-Hexadecylphenyl 2 - ethyl-hexyl maleate |
| Allyl esters of lard acids        | o-Tolyl 2 - octadecylcyclohexyl maleate   |
| Allyl naphthenate                 | Butyl methacrylate                        |
| Methallyl caproate                | o - Nonyphenyl - hexadecyl maleate        |
| Methallyl naphthenate             | Dihexadecyl maleate                       |
| Methallyl ricinoleate             | Di - methylcyclohexyl maleate             |
| Methallyl p-octylbenzoate         | Mono-2-ethylhexyl maleate                 |
| Methallyl oleate                  | Di-2-ethylhexyl maleate                   |
| Methallyl cyclohexane carboxylate | Di-dodecyl maleate                        |
| Methallyl palmitate               | Di-dodecyl fumarate                       |
| Crotyl oleate                     | Di-dodecyl mesaconate                     |
| Crotyl naphthenate                | Di-dodecyl citraconate                    |
| $\alpha$ -Methylcrotyl palmitate  | o-Tolyl octadecyl itaconate               |
| 1-propenyl naphthenate            | Mono-hexadecyl itaconate                  |
| 1-propenyl elaidate               | Isopropenyl palmitoleate                  |
| Dodecyl acrylate                  | 1-decenyl laurate                         |
| Hexadecyl methacrylate            | 1-hexadecenyl myristate                   |
| Isobutyl $\alpha$ -decylacrylate  |                                           |
| Vinyl p-n-octyl benzoate          |                                           |
| Allyl 3,5-diisobutyl benzoate     |                                           |
| Cyclohexyl methacrylate           |                                           |
| Cyclohexyl 2-dodecanoate          |                                           |

Although any of the oil-solubilizing compounds described above will give effective copolymer compositions for lubricant compositions in accordance with the present invention, alkyl esters of  $\alpha, \beta$ -unsaturated monocarboxylic acids of from 3 to 5 carbon atoms having alkyl groups of at least 4 carbon atoms and, more particularly, of from 8 to 30 carbon atoms are most preferred both for availability and effectiveness of copolymers prepared from them. Representative acids of this type are the acrylic, methacrylic, crotonic, tiglic, angelic,  $\alpha$ -ethylacrylic,  $\alpha$ -methylcrotonic,  $\alpha$ -ethylcrotonic,  $\beta$ -ethylcrotonic,  $\beta$ -propylcrotonic,

ic, and hydroxobic acids and the like. Even more desirable are the alkyl esters of acrylic and methacrylic acids and mixtures thereof containing an average of from 10 to 20 carbon atoms in the alkyl groups, since they are found to provide highly superior polymers for the lubricant compositions of the invention and are obtainable in commercial quantities.

The epoxy substituted monomeric components of the additives of this invention as already mentioned are preferably derivatives of a polymerizable oxirane compound which is reacted with an amino compound containing at least one nontertiary amino group. Suitable epoxy substituted monomers include the olefins, ethers and esters of the types mentioned above in connection with the oil-solubilizing monomers, the essential difference being that they are characterized by the presence of an epoxy group in addition to the polymerizable ethylenic group.

For present purposes the preferred epoxy compounds are the above-mentioned olefins, ethers and esters as illustrated by butadiene monoxide, allyl glycidyl ether, vinyl glycidyl ether, glycidyl methacrylate, diglycidyl maleate and the like. Such epoxy compounds when reacted with a single nontertiary amino group of an amino compound provide monomers having the following structure in addition to the polymerizable ethylenic group:



in which  $R_1$  is hydroxyalkyl, aminoalkyl or polyalkylene polyamine in structure and  $R_2$  is hydrogen or a group similar to group  $R_1$ . In the formulae  $R_1$  and  $R_2$  may also be present in the form of a single aromatic or cycloaliphatic ring as in the case of N-amino propyl morpholine, N-2-amino ethyl piperazine, etc.

Presently preferred are the reactants of glycidyl esters of unsaturated monocarboxylic acids of 3 to 5 carbon atoms and aliphatic polyamines such as alkylene diamines and polyalkylene polyamines in which the alkylene groups contain from 2 to 4 carbon atoms each and the polyalkylene polyamines contain from 2 to 8 alkylene amine units. The amino groups of the polyamines may have nitrogen atoms substituted by alkyl radicals of from 1 to 4 carbon atoms, so long as there is at least one primary or secondary amino group present for reacting with the epoxy ring of the glycidyl group. Representative amino compounds which can be reacted with the epoxy ring or the oxirane group as described above include:

## ALIPHATIC AMINES

|                                |                                             |
|--------------------------------|---------------------------------------------|
| Ethylene diamine               | N-oleamide of hydroxyethyl ethylene diamine |
| N,N-dimethyl propylene diamine | Diethylene triamine                         |
| 60                             |                                             |
| Ethanolamine                   | Tetraethylene pentamine                     |
| Amino ethyl ethanolamine       | N-amino ethyl stearyl imidazoline           |
| Diethanolamine                 |                                             |

## AROMATIC AMINES

|    |                            |                   |
|----|----------------------------|-------------------|
| 65 | N-2-amino ethyl piperazine | Phenylene diamine |
|    | N-amino propyl morpholine  |                   |

In preparing the polymers of the invention it is only necessary that conditions be chosen which ensure polymerization and the formation of polymers having the requisite oil-solubility and polarity. The oil-solubilizing (A) monomers vary somewhat in their solubilizing characteristics. Thus, in some cases it is possible to obtain polymers which are soluble in oil by employing oil-solubilizing (A) and glycidyl-amino compound (B) monomer

ratios as low as 1:1. In other cases it is advantageous to raise the ratio of (A) to (B) to a much higher value, for example, about 100:1 in order to obtain a polymer product having optimum oil-solubility and polarity characteristics. As a general rule, however, polymers having excellent dispersant characteristics together with the requisite oil-solubility (which should be at least 0.5 and is preferably as great as 10% by weight of the lubricant composition) can be prepared by employing oil-solubilizing (A) monomers to polar (B) monomers in ratios of from about 5:1 to 100:1 and such a range is preferably employed where possible.

Because of the variations in the types of oil-solubilizing (A) monomers and the polar (B) monomers as mentioned above, it is preferable to describe the overall composition of the polymers of this invention on the basis of amino nitrogen content of the (B) component. Suitable detergents or dispersants are obtained when this nitrogen content is from 0.05 to 8.0% by weight of the polymer. Preferably, the polymers contain from 0.1 to 5.0% by weight.

The macromolecules employed in the compositions of this invention can be prepared by any one of several methods as known in the art. As indicated above, the oil-solubilizing groups, the amino-alcohol groups and optional polar groups of the macromolecules are attached in various ways. In the case of the essential amino-alcohol groups there are three general methods of attachment. (1) The amino-alcohol group may be incorporated by reacting a preformed polymer containing reactive centers such as free carboxyl groups with glycidol following which the epoxy group of the glycidyl group is reacted with the amino compound. (2) The amino-alcohol group may also be introduced as the polymerizable monomer prepared by (a) reacting glycidol with a reactive monomer such as methacrylic acid which is then polymerized to give a glycidyl methacrylate containing copolymer in which the epoxy groups may be reacted with the amino compound or (b) reacting glycidol with a reactive monomer such as methacrylic acid followed immediately by reaction of the epoxy group of the glycidyl group with the amino compound to give the amino-alcohol group monomer which is then copolymerized with the oil-solubilizing (A) and optional (C) polar monomers. (3) The amino-alcohol group may be incorporated into a preformed polymer by reacting an epoxy amino compound reaction product of the amino-alcohol group type mentioned above with reactive centers as described in (1). In this case the epoxy portion of the glycidyl group has already been reacted with the amino compound. Thus, it may be seen that one may polymerize a mixture of the desired monomer components to form the polymer or the copolymers may be obtained by starting with suitable precursor compounds with the desired monomer units and treating the intermediate to obtain the desired final product.

In all of the above general methods, when the oxirane ring is reacted with the amino compound, a large excess of amine is employed to prevent cross linking. When the oxirane ring is opened with an amino compound, a new amine and a free hydroxyl group are formed as follows:



When  $\text{R}_1$  or  $\text{R}_2$  is hydrogen, these hydrogen atoms, as well as those of an other nontertiary amino group are capable of opening a second oxirane ring. This may result in cross-linked, resinous polymers. For example, in the case where the amino group is added to the monomer before polymerization (as in method 2b above) there would result a di-ethylenically unsaturated monomer which would necessarily cross link during polymerization. To avoid these undesirable reactions, and ensure

linear oil-soluble polymers, a large excess of amine is employed. This forces the desired reactions. Excess amine is readily removed by distillation, precipitation or any other conventional separation process. Such excesses are usually at least three- to five-fold and range as high as 10 to 30 times the theoretical amount required to react one mole of amino-compound with one mole of epoxy compound, particularly in the case of the more readily cross-linked primary amino and polyamino compounds.

When the polymeric additive of this invention, or a suitable polymeric intermediate, is to be prepared by reaction of monomeric components, said polymers can be prepared by conventional bulk, solution or emulsion methods in the presence of an addition polymerization initiator.

Preferably, however, the copolymerization is effected in an inert organic solvent such as benzene, toluene, xylene or petroleum naphtha in the presence of a free radical-liberating type of initiator such as a peroxy compound, for example, benzoyl peroxide, acetyl peroxide, 20 butyl hydroperoxide, di-tert. butyl peroxide, di-benzoyl peroxide, or di-tert. amyl peroxide, or an azo initiator such as 1,1'-azodicyclohexane, carbonitrile or  $\alpha,\alpha'$ -azodiisobutyronitrile. The catalyst, or polymerization initiator, can be employed in an amount of from about 0.01 to 10%, with a preferred range being from 0.01 to 2%. If desired, the catalyst can be added in increments as the reaction proceeds. Likewise, additional portions of the solvent can also be added from time to time in order to maintain the solution in a homogeneous condition. The temperature of copolymerization varies from about 100 to 300° F. with the optimum temperature for any given preparation depending on the nature of the solvent, the concentration of monomers present in the solvent, the catalyst and the duration of the reaction. Much the same conditions are employed when the copolymerization is effected in bulk rather than in the presence of an inert solvent.

The additives of this invention have apparent molecular weights as determined by standard light scattering methods and viscosity measurements of at least 2,000 and preferably at least 50,000. For practical purposes molecular weights of from 100,000 to 1,000,000 are most suitable from the standpoint of viscosity and other physical characteristics of the polymeric additives.

The following examples are illustrative of typical methods for preparing the alcohol-amino compound polymeric type additives according to the invention.

#### Example 1

This example illustrates the preparation of a copolymer intermediate of mixed dodecyl and octadecyl methacrylates with glycidyl methacrylate.

A 2-liter flask fitted with stirrer, reflux condenser and dropping funnel is charged with 750 g. (2.5 moles) of alkyl methacrylate in which the alkyl groups are a mixture of 60% by weight dodecyl and 40% by weight octadecyl groups, 14.2 g. (0.1 mole) glycidyl methacrylate and 510 g. benzene. The flask is purged with nitrogen. The charge mixture is heated to reflux and is polymerized for about 7 hours by the addition of a 2% solution of bis-azoisobutyronitrile in benzene as catalyst. The catalyst is added at a rate of 3.8 ml. every 15 minutes.

The polymer formed in the above reaction is precipitated from the reaction mix by the addition of a four-fold volume of acetone. The yield of polymer is 690 g. which is equivalent to 90.3% of theoretical based on the reactants. A determination of the oxirane oxygen of the epoxy groups in the glycidyl portion was made of the product in the acetone phase. This determination indicates the presence of 1.5 g. or 10.5% by weight of glycidyl methacrylate. Accordingly, the alkyl meth-

acrylate and glycidyl methacrylate are present in a 25:1 mole ratio.

*Example 2*

This example shows the conversion of the alkyl methacrylate and glycidyl methacrylate copolymer intermediate of the above preparation to glycidyl-amino compound.

In a 2-liter flask, as described above, 76 g. of the copolymer of Example 1 is dissolved in 200 ml. of xylene. This solution is refluxed for 5 hours with 20 g. N,N - dimethyl - 1,3 - propane diamine. The polymeric product is precipitated from xylene solution three times with methanol. A nitrogen determination shows 0.33% nitrogen which agrees with a theoretical of 0.36% nitrogen for a copolymer of alkyl methacrylate (60% dodecyl and 40% octadecyl) and glycidyl methacrylate-N,N-dimethyl-1,3-propane diamine of 25:1 mole ratio.

Other polymers illustrative of the compositions of the invention are also prepared according to the general procedures outlined in the above discussion and examples. These polymers are described with respect to the particular monomers and mole ratios employed, along with pertinent performance data, in the tables which appear below.

In general, excellent detergent and anti-wear properties can be imparted to lubricating oils by dissolving therein a quantity of from about 0.1 to 10% by weight of the polymers of the type described above, although a preferred range is from about 1 to 5% by weight. On the other hand, since the polymers of this invention are unusually compatible with mineral and other lubricating oils in substantially all proportions, as much as 75% of the present polymer additives can be dissolved in a suitable lubricating oil for the purpose of preparing a concentrate capable of dilution with lubricating oils and the like to prepare the final lubricant composition. Such concentrates, which may also contain other additives in desired amounts, and which normally contain at least 10% of the polymer, comprise a convenient method for handling the polymer and may be used as a compounding agent for lubricants in general.

The polymeric additives of this invention can be used with good effect in the case of any one of a wide variety of oils of lubricating viscosity, or of blends of such oils. Thus, the base oil can be a refined Pennsylvania or other paraffin base oil, a refined naphthenic base oil, or a synthetic hydrocarbon or nonhydrocarbon oil of lubricating viscosity. As synthetic oils there can be mentioned alkylated waxes and similar alkylated hydrocarbons of relatively high molecular weight, hydrogenated polymers of hydrocarbons, and the condensation products of chlorinated alkyl hydrocarbons with aryl compounds. Other suitable oils are those which are obtained by polymerization of lower molecular weight alkylene oxides such as propylene and/or ethylene oxide. Still other synthetic oils are obtained by etherification and/or esterification of the hydroxy groups in alkylene oxide polymers such as, for example, the acetate of the 2-ethylhexanol-initiated polymer of propylene oxide. Other important classes of synthetic oils include the various esters as, for example, di-(2-ethylhexyl)sebacate, tricresyl phosphate and silicate esters. If desired, the oil can be a mixture of mineral and synthetic oils.

While satisfactory lubricant compositions can be obtained by adding to the base oil employed only one or more of the polymeric additives of the type described above, it also falls within the purview of this invention to provide lubricant compositions which contain not only such polymers, but also other additives such as pour point depressants, oiliness and extreme pressure agents, anti-oxidants, corrosion inhibiting agents, blooming agents, thickening agents and/or compounds for enhancing the temperature-viscosity characteristics of the oil. The present invention also contemplates the addition to the lubricant composition (particularly when the amount

of copolymer employed is relatively small) of auxiliary detergents and/or antiwear agents.

Illustrative lubricant compositions of the above type containing the copolymeric additives of the invention in combination with other agents may include, for example, from about 0.1 to 10% by weight of alkaline earth metal higher alkylphenate detergent and wear reducing agents such as calcium alkylphenates having an average of approximately 14 carbon atoms in the alkyl group as well as organic thiophosphate corrosion and high temperature oxidation inhibitors such as the reaction product of pinene and  $P_2S_5$  and the bivalent metal dihydrocarbyl dithiophosphates, zinc butyl hexyl dithiophosphate and zinc tetradecylphenyl dithiophosphate in amounts of from about 0.1 to 10% by weight of the composition. Temperature-viscosity improving agents which may be employed in the compositions, usually in amounts of from about 1 to 10% by weight, include by way of example the homopolymers of alkyl methacrylates such as the dodecyl methacrylate polymers known to the trade as Acryloid 710 and Acryloid 763, products of Rohm & Haas Company, and high molecular weight butene polymers such as Paratone ENJ 15P, a product of the Enjay Company.

The polymeric additives of the invention as described above are evaluated as detergents in lubricating oils and as dispersants in hydrocarbon liquids in a number of tests. The results of the tests along with a description of the polymeric additives are set out in the following tables.

In the tests as described below the base oil, unless otherwise specified, is a solvent refined wax free 150 Neutral mineral lubricating oil. It has a viscosity index of 88 and is derived from California waxy crude. The polymeric additive is employed in the oil in an amount of 2.8% by weight of polymer based on total composition, unless otherwise noted.

In the test where the piston varnish ratings are obtained, a given lubricating oil composition is tested as the crankcase lubricant in a 6-cylinder Chevrolet engine using a low grade gasoline especially prone to cause engine deposits, the conditions being those defined in the standard FL-2 test procedure as described in the June 21, 1948, report of the Coordinating Research Council. This procedure requires the maintenance of a jacket temperature of 95° F. and a crankcase oil temperature of 155° F. at 2500 r.p.m. and 45 brake horsepower of 40 hours, and therefore closely simulates the relatively "cold" engine conditions which are normally experienced in city driving. At the end of each test, the engine is dismantled and the amount of engine deposits on the piston determined and expressed as the piston varnish rating. This value is obtained by visually rating (on a scale of 0 to 10, with 10 representing the absence of any deposit) the amount of deposit on each piston skirt and averaging the individual ratings so obtained for the various pistons. Under the conditions of this test, a piston varnish rating of 3.5 is indicative of detergent performance, though preferably this rating should be 4 or above. In the case of the base oil alone without the addition of any additives it is found that the piston varnish rating is approximately 3.0. On the other hand, as indicated by the data presented in the tables below, when the base oil is compounded with the indicated amounts of a copolymer, greatly superior results are obtained.

The polymeric additives according to the invention are also evaluated for their dispersing properties in the standard Carbon Peptization Test. In this test 0.1 g. of 100% active copolymer is dissolved in 100 ml. of kerosene in a 100 ml. graduated glass cylinder. To this solution of polymer is added 0.5 g. of ordinary lamp black. The contents of the graduated cylinder are mixed by manual shaking using an end-over-end motion for exactly one minute. After the shaking, the cylinder is placed upright and observed periodically about every half hour.

The Carbon Peptization Test number (CPT) is expressed as hours required for total settling of the carbon black.

4, 8 and 11 contain no amino compound, as indicated in the table.

TABLE I

| Ex. No. | Amino Compound Of (B) Monomer | Molar Ratio of Monomers | Percent N | V.I. | PD No. (L-1)  | PVR (FL-2) | CPT (Hours) |
|---------|-------------------------------|-------------------------|-----------|------|---------------|------------|-------------|
| 3       | None                          | 5/1                     |           | 88   | 800, 800, 800 | 3.0        | <1          |
| 4       | None                          | 5.9/1                   | 0.64      | 148  |               |            | 2           |
| 5       | Di-n-hexyl-amine              | 5.9/1                   | 0.59      | 150  |               |            | 22          |
| 6       | Ethanolamine                  | 6.8/1                   | 0.59      | 152  |               |            | 20          |
| 7       | N-aminoethyl ethanolamine     | 5.9/1                   | 1.42      | 156  |               |            | 48          |
| 8       | None                          | 10/1                    |           |      |               | 3.2        | 1           |
| 9       | Dimethyl amino propylamine    | 10/2                    | 0.86      | 141  | 40, 0, 0      | 4.4        | 24          |
| 10      | Tetraethylene pentamine       | 10/0.9                  | 1.83      |      |               | 4.5        | 30          |
| 11      | None                          | 25/1                    |           |      |               |            | 3           |
| 12      | Amino ethyl piperazine        | 25/1                    | 0.23      | 143  |               |            | 6           |
| 13      | Diethylene triamine           | 25/1                    | 0.58      | 141  |               |            | 8           |
| 14      | Dimethyl amino propylamine    | 33/1                    | 0.28      |      |               | 4.9        | 30          |
| 15      | Tetraethylene pentamine       | 30/1                    |           |      |               |            | 17          |

A CPT of 4 hours or more indicates significant dispersing properties. The Carbon Peptization Tests are found to correlate well with the FL-2 engine test described above.

In addition to the foregoing tests of detergency and dispersing properties of the polymeric additives data were also obtained in a Caterpillar L-1 test under Supplement I conditions for a period of 120 hours as described in the Coordinating Research Council Handbook, January 1946.

In these tests the PD numbers of oils are obtained to

30 number.

In Table II below, additional examples are given to show several typical variations of the primary components of the novel amino-alcohol copolymers according to this invention. Different oil-solubilizing monomers are included and the characteristic amino-alcohol groups are incorporated in a variety of forms, such as those derived from olefins and ethers. The effectiveness of the copolymers is illustrated by their Carbon Peptization Test

TABLE II

| Ex. No. | Oil-Solubilizing (A) Monomer                            | Alcohol-Amino (B) Monomer                                                                          | Molar Ratio of Monomers | Percent N | CPT (Hours) |
|---------|---------------------------------------------------------|----------------------------------------------------------------------------------------------------|-------------------------|-----------|-------------|
| 16      | {60% Dodecyl methacrylate<br>40% Octadecyl methacrylate | {Allyl glycidyl ether-Tetra-<br>ethylene pentamine<br>Allyl glycidyl ether-3,4-<br>Diamino toluene | 8.9/1                   | 2.2       | 18          |
| 17      | {40% Dodecyl methacrylate<br>60% Octadecyl methacrylate | Butadiene monoxide-<br>2-Amino ethyl piperazine                                                    | 70/1                    | 0.14      | 5           |
| 18      | {60% Dodecyl methacrylate<br>40% Octadecyl methacrylate | Butadiene monoxide-<br>Diethylene triamine                                                         | 19/1                    | 0.48      | 7           |
| 19      | {60% Dodecyl methacrylate<br>40% Octadecyl methacrylate | Butadiene monoxide-<br>Allyl glycidyl ether-Dimethyl<br>amino propylamine                          | 10.5/1                  | 1.3       | 8           |
| 20      | Vinyl stearate                                          | Allyl glycidyl ether-Dimethyl<br>amino propylamine                                                 | 20/1                    | 0.43      | 16          |
| 21      | {50% Vinyl acetate<br>50% Didodecyl maleate             | Allyl glycidyl ether-Dimethyl<br>amino propylamine                                                 | 32/1                    | 1.18      | 16          |

show the piston discoloration rating. Following each engine test the three piston lands are examined visually. A piston land which is completely black is assigned a PD number of 800. The piston lands which are completely clean are assigned a PD number of 0. Intermediate PD numbers are assigned in proportion to the extent and degree of discoloration of the piston lands.

In Table I below the polymers all contain a representative oil-solubilizing (A) monomer consisting of 60% by weight dodecyl methacrylate and 40% by weight of octadecyl methacrylate. The glycidyl component of the (B) monomer in the polymer is glycidyl methacrylate, which is also representative of such components. In the examples of the table a variety of amino compounds are shown which are reacted with the epoxy group of the glycidyl methacrylate. The polymers of the examples also are identified by their monomer ratios, as well as by analysis for nitrogen on a percent by weight basis (percent N). The Viscosity Index of the oils in the examples is also shown in the table as evidence of the important viscosity-temperature characteristics of the lubricant compositions containing polymers according to this invention.

In the examples of the table the performance of the base oil alone, without any polymers whatsoever, is shown as Example No. 3. The copolymers of Examples Nos.

From the tests of the foregoing tables it will be seen that each of the illustrative compositions containing the polymeric lubricating oil additives according to the invention possesses greatly improved lubricating properties compared to the base oils alone, or oils containing other closely related copolymers. The copolymeric additives containing alcohol-amino constituents are remarkably effective detergents and dispersants. Significant benefits are obtained in both low temperature type of engine operation as found in gasoline internal combustion engines and in high temperature type of operation as found in diesel engines. The combination of such low and high temperature detergent and dispersant properties in lubricant compositions containing a single polymeric additive is particularly important. The presence of both desirable properties in a single polymeric additive facilitates the provision of a single lubricating oil composition suitable for use in either gasoline engine lubricating oils or diesel engine lubricating oils.

We claim:

70 1. A detergent oil-soluble copolymer of (A) at least one alkyl methacrylate having 8 to 30 carbon atoms in the alkyl group and (B) glycidyl methacrylate, the mole ratio of (A) to (B) being from about 5:1 to 100:1, said polymer being reacted with N-aminoethyl ethanolamine, 75 the molar ratio of the glycidyl portion to N-aminoethyl

11

ethanolamine being approximately 1:1, said copolymer containing from about 0.05 to 8% by weight of nitrogen and having a total molecular weight of at least about 2000, said copolymer being characterized by a solubility in mineral lubricating oil of at least 0.5% by weight.

2. A lubricant composition comprising a major portion of an oil of lubricating viscosity and a minor portion sufficient to enhance the detergent characteristics of the composition of the detergent oil-soluble copolymer of claim 1.

12

## References Cited by the Examiner

## UNITED STATES PATENTS

|           |      |                   |       |          |
|-----------|------|-------------------|-------|----------|
| 2,582,708 | 1/52 | Lippincott et al. | ----- | 252—56   |
| 2,737,496 | 3/56 | Catlin            | ----- | 252—51.5 |
| 2,761,870 | 9/56 | Payne et al.      | ----- | 260—348  |
| 2,781,335 | 2/57 | Cupery            | ----- | 260—85.7 |
| 2,949,445 | 8/60 | Blake             | ----- | 260—86.1 |

10 DANIEL E. WYMAN, Primary Examiner.